

## UNITED STATES PATENT OFFICE

2,307,307

## EXTREME PRESSURE LUBRICANT

Bernard H. Shoemaker, Hammond, Ind., assignor  
to Standard Oil Company, Chicago, Ill., a cor-  
poration of Indiana

No Drawing. Application September 12, 1938,  
Serial No. 229,523

11 Claims. (Cl. 252—46)

This invention relates to improvements in lub-  
ricants, and in particular, to improvements in  
extreme pressure lubricants adapted for use on  
bearing surfaces which are subjected to high  
pressures and high rubbing velocities during use.

High unit pressures which are encountered  
frequently in devices employed for the trans-  
mission of power, such as hypoid gears, worm  
gears, heavy duty bearings, planetary automatic  
shifts and the like, necessitate the use of lubri-  
cants having superior load carrying properties.  
Lubricants possessing superior load carrying  
properties, which make them specially adapted  
for use under conditions of high pressure where  
the pressures encountered are of such magnitude  
that the separation of gear teeth or bearing sur-  
faces by an ordinary oil film is not possible, are  
known in the art as extreme pressure lubricants.  
Extreme pressure lubricants are likewise impor-  
tant in cutting and drawing operations where the  
oil must withstand the high pressures encoun-  
tered under those conditions of use.

It is an object of this invention to provide an  
improved extreme pressure lubricant which will  
give superior lubrication to bearing surfaces  
which are subjected to high pressures and/or  
high rubbing velocities.

Another object of this invention is to provide  
a lubricant which will prevent gear teeth or bear-  
ing failure from scoring or galling caused by the  
welding of small areas of the mating surfaces  
due to high pressure and high temperature.

I have found that the foregoing objects can be  
attained if small amounts, preferably from about  
0.01% to about 2%, of thioketopolysulfides, of  
the type obtained by reacting an alkali-metal  
xanthate with a sulfur chloride, are added to  
lubricants, such as oils and greases. These com-  
pounds have the general formula  $(RXC=S)_2S_n$ ,  
in which R is a radical selected from the group  
consisting of alkyl, chloralkyl, aryl and chloraryl  
radicals, X is an element selected from the group  
consisting of oxygen and sulfur, and n is an in-  
teger greater than 2.

These compounds may be prepared by react-  
ing an alkali metal xanthate with a sulfur chlo-  
ride. For example, the tetrathio derivative may  
be prepared by reacting twenty-eight grams of  
potassium ethyl xanthate, suspended in hexane,  
or any other suitable diluent, with a little less

than the calculated required amount of  $S_2Cl_2$ ,  
and refluxing the reactants on a steam bath for  
about two hours. The following reaction is be-  
lieved to take place:



To obtain the trithio derivatives the alkali metal  
xanthate is reacted with  $SCl_2$ .

Because of the presence of the thio-keto group



15 in these compounds I have called them thioketo-  
polysulfides, but more specifically I believe them  
to be thioformate polysulfides, and while I refer  
to them hereinafter as thioformates, I do not wish  
to limit the scope of this invention to thioform-  
ates, but to the reaction product of an alkali-  
metal xanthate and a sulfur chloride.

Specific examples of the type of compounds  
which I may use are the following:

Tetrathio diethylthioformate  
Tetrathio dibutylthioformate  
Tetrathio diamyldithioformate  
Tetrathio dilaurylthioformate  
Tetrathio dilauryl dithioformate  
Tetrathio dichlorbutylthioformate  
Tetrathio dichlorlauryldithioformate  
Tetrathio diphenylthioformate  
Tetrathio dichlorphenyldithioformate  
Trithio dipropylthioformate  
Trithio dichlorbutylthioformate  
Trithio diphenylthioformate  
Trithio di-octyldithioformate

40 I have found that small amounts of these com-  
pounds added to lubricating oils and greases pro-  
vide lubricants which enable the bearing surfaces  
to withstand high pressures and high lubricating  
velocities without noticeable wear. Similarly,  
these compounds may be compounded with draw-  
ing and/or cutting lubricants.

45 The load carrying capacity of extreme pres-  
sure lubricants may be determined by extreme  
pressure testing machines such as the Almen  
testing machine described by Wolf and Mourey  
in their paper on "Extreme Pressure Lubricants"  
given at the 13th annual meeting of the A. P. I.

at Houston, Texas, November 17, 1932. Briefly, it consists of a test pin or journal made of  $\frac{1}{4}$  inch diameter drill rod which can be rotated in a  $\frac{1}{2}$  inch long split bushing with provisions for loading the bearing thus formed by clamping together the two halves of the split bushing. Provision is also made to measure the torque required to rotate the journal in the loaded bearing.

The standard method of making a test on the Almen machine consists in immersing the test pin and bushings in the lubricant to be tested and then rotating the test pin at 600 R. P. M. The load, which clamps the two halves of the split bushing, is increased at the rate of 2 lbs. added every 10 seconds. A record is made of the torque required to rotate the pin at each load increment and the test is completed either when 30 lbs. have been added to the loading device or when seizure occurs, whichever happens first.

The following example will illustrate the effectiveness of the addition of small amounts of thioketo polysulfides in lubricating oils under extreme pressure conditions. A mineral lubricating oil having a viscosity of about 170 seconds at 130° F. and the same oil with 0.5% of tetrathio diethylthioformate when tested in the Almen testing machine gave the following results:

|                                           | Load at which seizure occurred |        |
|-------------------------------------------|--------------------------------|--------|
|                                           | Pounds                         | Pounds |
| Control                                   | 16                             | 6      |
| Control+0.5% tetrathio diethylthioformate | 30                             | 30+    |

While I have described my invention with a specific embodiment thereof, it is to be understood that the same is merely illustrative of the invention and not a limitation thereof, except insofar as the same is defined in the appended claims, which are to be interpreted as broadly as the prior art will permit.

I claim:

1. An extreme pressure lubricant containing a lubricant and a thioketo polysulfide having the general formula  $(RXC=S)_2S_n$  in which R is a radical selected from the group consisting of alkyl, chloralkyl, aryl and chloraryl radicals, X is an element selected from the group consisting of oxygen and sulfur and n is an integer greater than 2, said thioketo polysulfide being used in small but sufficient quantities to impart extreme pressure properties to said lubricant.

2. An extreme pressure lubricant containing a

mineral lubricating oil and from about 0.01% to about 2% of a thioketo polysulfide having the general formula  $(RXC=S)_2S_n$  in which R is a radical selected from the group consisting of alkyl, chloralkyl, aryl and chloraryl radicals, X is an element selected from the group consisting of oxygen and sulfur and n is an integer greater than 2.

3. An extreme pressure lubricant containing a mineral lubricating oil and from about 0.01% to about 2% of tetrathio diethylthioformate.

4. An extreme pressure lubricant containing a lubricant and a thioketo polysulfide having the general formula  $(RXC=S)_2S_3$  in which R is a radical selected from the group consisting of alkyl, chloralkyl, aryl and chloraryl radicals, and X is an element selected from the group consisting of oxygen and sulfur, said thioketo polysulfide being used in small but sufficient quantity to impart extreme pressure properties to said lubricant.

5. An extreme pressure lubricant containing a lubricant and a thioketo polysulfide having the general formula  $(RXC=S)_2S_4$  in which R is a radical selected from the group consisting of alkyl, chloralkyl, aryl and chloraryl radicals, and X is an element selected from the group consisting of oxygen and sulfur, said thioketo polysulfide being used in small but sufficient quantity to impart extreme pressure properties to said lubricant.

6. An extreme pressure lubricant containing a lubricant and a tetrathio alkyl thioformate in small but sufficient quantity to impart extreme pressure properties to said lubricant.

7. A lubricating composition comprising a lubricating oil base stock and at least .01% of a soluble xanthogen sulfide having the general formula:



where R and R' are like or unlike alkyl or aryl radicals, and X is either oxygen or sulfur.

8. A composition of matter comprising an oil and a small amount of organic xanthogen tetrasulfide.

9. A lubricating composition comprising a mineral lubricating oil and at least about 0.01% of a soluble organic xanthogen tetrasulfide.

10. A lubricating composition according to claim 9 in which the tetrasulfide is an alkyl xanthogen tetrasulfide.

11. A lubricating composition according to claim 9 in which the tetrasulfide is ethyl xanthyl tetrasulfide.

BERNARD H. SHOEMAKER.